

T. MIDGLEY.  
METHOD OF COATING FABRIC.  
APPLICATION FILED MAR. 18, 1919.

1,323,606.

Patented Dec. 2, 1919.

2 SHEETS—SHEET 1.



INVENTOR.  
Thomas Midgley.  
BY Chapin Mal.  
ATTORNEYS.

T. MIDGLEY.

METHOD OF COATING FABRIC.  
APPLICATION FILED MAR. 18, 1919.

1,323,606.

Patented Dec. 2, 1919.

2 SHEETS—SHEET 2.



# UNITED STATES PATENT OFFICE.

THOMAS MIDGLEY, OF SPRINGFIELD, MASSACHUSETTS, ASSIGNOR TO THE FISK RUBBER COMPANY, OF CHICOPEE FALLS, MASSACHUSETTS, A CORPORATION OF MASSACHUSETTS.

## METHOD OF COATING FABRIC.

1,323,606.

Specification of Letters Patent.

Patented Dec. 2, 1919.

Application filed March 18, 1919. Serial No. 283,368.

To all whom it may concern:

Be it known that I, THOMAS MIDGLEY, a citizen of the United States of America, residing at Springfield, in the county of 5 Hampden and State of Massachusetts, have invented certain new and useful Improvements in Methods of Coating Fabric, of which the following is a specification.

My invention relates to the manufacture 10 of rubber-coated fabric intended primarily for use in automobile tires. In its specific embodiment, it relates to the manufacture of so-called "cord fabric", which is a weftless fabric composed of a plurality of spaced 15 parallel cords held together by a coating of rubber. My invention may also be utilized in coating what is known as "thread fabric" composed of a warp of closely spaced parallel cords with a weft of widely spaced 20 threads; or in coating any sheet material.

My invention has for its object an improvement in the process of applying rubber to such fabrics.

Briefly it consists in applying a coating 25 of rubber and some solvent to a carrier surface having the property of adhering to such coating while the solvent is present, but losing that adherence when the solvent is dried out. The fabric, or plurality of parallel 30 cords if a cord fabric is being manufactured, is brought into contact with the coating, and the solvent is then dried out. The coated fabric is then in a condition to be separated from the carrier, which may be 35 used repeatedly. My invention will now be described with reference to the accompanying drawings, in which—

Figure 1 is an elevation, partly in section, 40 of one form of apparatus for carrying out my invention;

Fig. 2 is a perspective view of the comb used in guiding the parallel cords in the manufacture of cord fabric;

Fig. 3 is an enlarged cross section corresponding to Fig. 1 showing the carrier with the rubber coating thereon and the cords being embedded in the coating;

Fig. 4 is a section on line 4—4 of Fig. 3;

Fig. 5 is a perspective view showing the 50 coated fabric being stripped from the carrier;

Fig. 6 is a detail showing an adaptation of the apparatus of Fig. 1 for use with thread or woven fabric;

Fig. 7 is a diagrammatic view showing a modified form of apparatus; and

Fig. 8 is a diagrammatic view of a further modification.

In the embodiment of my invention illustrated in Fig. 1, a plurality of cords 10 are led from a creel 11, which is of the usual form, between guides 12, here shown in the form of rollers. These guides serve to bring the cords into the same plane, and prevent one cord riding over an adjacent one when they are wound up with the carrier strip. Mounted beyond the guides 12, as on a shaft 13, is a comb indicated generally by 14. As shown in Fig. 2, the comb is formed of a frame 15 with small plates or slats 16, preferably of metal, mounted transversely thereof, leaving slots between them, through each of which a single cord is guided.

Carried on a pedestal 17 is a roll 18 of glazed fabric or holland 19, which passes over an idler 20 and over a coating roll 21 located in a tank 22, filled with rubber cement. After the holland has thus received a coating of rubber cement 23 on both sides, it is led around a roll 24 adjacent the comb 14. The cords are attached to the holland in any convenient way, and the roll 24 is rotated, as by a pulley 25, thus winding the parallel cords and the holland together on the roll. In this way, the layers of cords 26 are inclosed between successive coated layers of holland, thus applying a coat of rubber cement to each side of the cords. It will be noticed that the comb is located quite close to the roll 24. This is important in order to preserve a spacing between the parallel cords as they are laid on the coated holland. If there is a considerable distance between the comb and roll the cords are likely to close up on one another, having insufficient separation to allow of the rubber passing up between the cords. The cords are thus not only made up into a compound sheet composed of a layer of cords coated on either side by rubber, but the cords are firmly embedded in a matrix of rubber. This would not be the case if the cords passed through any substantial distance between the comb and the roll, as in this case they would tend to bunch.

When the holland and cords have been wound up to the desired size the cords are severed, taking due precaution to prevent

the cords losing their parallel relation, and the roll 24 removed and placed in a drier. After the rubber cement has thoroughly dried the cords with the rubber adhering thereto, and forming what may be termed a weftless fabric 26, can be stripped from the holland, which is capable of repeated use as a carrier.

If it is desired to treat thread fabric or 10 ordinary woven fabric instead of the parallel cords the same procedure may be followed, omitting the comb, as illustrated in Fig. 6. This same modification may be adopted with reference to Figs. 7 and 8 described below.

In Fig. 7 is illustrated means for carrying out my invention using an endless carrier 27, of holland or sheet metal. This is led over rolls 28, 29, and 30, and over a 20 coating wheel 31 running in a tank 32 containing rubber cement, being thereby coated on one side only. Cords 33 are led from a creel 34 between guides 35 and through a comb 36, joining the endless carrier over roll 29. The carrier and cords then pass over a heater 37, the length of which is sufficient to thoroughly dry out the cement, and the resulting cord fabric 38, composed of the cords and the coating carried by the 30 endless band, is wound up on a reel 39. To prevent adhesion of the layers of cord fabric a separating strip or liner 40 may be fed in from a reel 41. A suction hood 42 is provided over the heater to remove the 35 vapors and hasten the drying. This method has the advantages of reducing the amount of holland necessary to be kept on hand, and reducing time and labor by drying and peeling the fabric from the carrier continuously with the step of associating the cords with the carrier.

In Fig. 8 a large drum 43 is substituted for the carrier strip of the other forms. This drum receives a sheet of rubber cement 44 from a roll 45 immersed in a tank 46. Cords 47 are led from a creel 48, between guides 49, and through comb 50 as before, and travel over the upper surface of the drum in contact with the sheet of cement. 50 The drum is heated, as by steam admitted through a pipe 51 and a hollow axle 52 of the drum, and the temperature and speed of rotation are adjusted so that the rubber cement will be dried by the time the opposite side of the drum is reached. At this

point the cord fabric 53, composed of the sheet of cement 44 and cords 47, is stripped from the drum and wound on a reel 54. As before, a liner 55 may be introduced from a reel 56 if desired.

It will be understood that the specific means illustrated are not the only ones by which my invention may be carried out, and I do not limit myself thereto.

What I claim is—

1. The method of impregnating and coating fabric, consisting in coating a carrier strip of glazed fabric with rubber cement, bringing the fabric to be coated into contact with the rubber coating, rolling the carrier strip and fabric together, drying, and stripping the fabric and rubber from the carrier strip.

2. The method of forming a weftless cord fabric, consisting in coating a carrier with rubber cement, bringing a plurality of spaced parallel cords into contact with the rubber coating, drying, and stripping the cords and rubber from the carrier.

3. The method of forming a weftless cord fabric, consisting in coating a carrier strip of glazed fabric with rubber cement, bringing a plurality of spaced parallel cords into contact with the rubber coating, drying, and stripping the cords and rubber from the carrier.

4. The method of forming a weftless cord fabric, consisting in coating a carrier strip of glazed fabric with rubber cement, bringing a plurality of spaced parallel cords into contact with the rubber coating, rolling the carrier strip and fabric together, drying, and stripping the cords and rubber from the carrier strip.

5. The method of forming a weftless cord fabric, consisting in coating a carrier with rubber cement, bringing a plurality of spaced parallel cords into contact with the coating, drying, stripping the cords and rubber from the carrier, and giving the fabric thus resulting a further coating of rubber.

6. In a device for producing a weftless cord fabric, a carrier, means for coating the carrier with rubber cement, a supply for a plurality of parallel cords, and a comb arranged close to the carrier to guide the cords into contact therewith and preserve them in parallel relation.

THOMAS MIDGLEY.